

H.T. Buffington, Jr.

Pile for Wrought-Iron Beams.

No 82,487.

Patented Sept 29, 1868.



Witnesses

Edward McPhee  
W.H. Becker

Inventor

H.T. Buffington  
by Forbush &  
Hargrave

# United States Patent Office.

HENRY T. BUFFINGTON, JR., OF BUFFALO, NEW YORK.

*Letters Patent No. 82,487, dated September 29, 1868.*

## IMPROVED FAGOT FOR BEAM.

The Schedule referred to in these Letters Patent and making part of the same.

TO ALL WHOM IT MAY CONCERN:

Be it known that I, HENRY T. BUFFINGTON, Jr., of the city of Buffalo, county of Erie, and State of New York, have invented a certain new and improved "Pile or Fagot for Wrought-Iron Beams;" and I do hereby declare that the following is a full, clear, and exact description thereof, reference being had to the accompanying drawings, making a part of this specification, in which—

Figure I is a cross-section of my improved "pile."

Figure II is a side elevation.

Figure III is a plan of same.

The nature of my invention consists—

First, in so arranging and combining the several pieces forming the pile as that the web, or the middle plate or plates thereof, shall pass through and entirely divide the flange-pieces, whereby the outward spreading of the flanges is prevented, and a more perfect welding of the flange-pieces to the web secured than in other known forms of "fagots."

Second, in forming the web of sectional plates, having their fibre running transversely, and extending through and dividing the flange-pieces, in combination with longitudinal side binding-plates filling between the flanges, said crossing of the fibre giving a stronger and more perfect beam.

Third, in forming T-ends on one, two, or more of the cross-web plates, so that they may act as binders, to hold the flange-pieces to the longitudinal side plates.

Like letters refer to like parts in each of the figures.

The web of the beam is composed of the middle cross-plates A, and side binding-plates B, while the flanges are composed of the form-bars C.

The middle plates A are arranged with their fibre running transversely through the pile, their outer ends being flush with the outside of the flange-pieces, and entirely separating the same.

The side binding-plates B run longitudinally, so that their fibre crosses that of the middle plates A. The flanges are placed upon the middle plate, and the side plates fill in between them, the inner sides of the flanges being rebated, as shown at D, to receive the edges of the side plates.

One or more of the cross-plates A is furnished with a T-head at each end, as shown at E, which laps over on to the flanges, and holds them against the side plates, thus holding the pile together in the direction of its depth.

At F are shown clamps, applied to the ends of the pile, and binding the side plates together, thus securing the pile in the direction of its breadth.

In charging the pile in the furnaces, it should be laid on its side, in which position all its parts are held firmly together. It is also in this position that it is passed through the "rolls."

It will be observed that the principal lines upon which the flanges weld to the web are at right angles to the direction of the pressure received in passing through the rolls, and that in consequence the welds must be of the most perfect character. This fact is due to the extension of the middle web through the flanges. In other piles of which I have knowledge, the principal lines upon which the flanges weld to the web are parallel to the direction of pressure, by reason of the contiguous flanges being formed in one plate, against the centre of which the web abuts, so that the rolls cannot exert an efficient pressure to produce the welds, and they are consequently often imperfect.

The crossing of the fibre of the web also insures the soundness of the beam, and increases its strength.

Having thus described my invention, what I claim, and desire to secure by Letters Patent, is—

1. The sectional web-plates A, arranged with their fibre's running transversely through the pile in combination with the longitudinal side binding-plates B, as and for the purpose set forth.

2. The cross clamp-plates, provided with the T-heads E, in combination with the flange-pieces C, and side binding-plates B, as and for the purpose set forth.

HENRY T. BUFFINGTON, JR.

Witnesses:

EDWARD WILHELM,  
V. H. BECKER.